

1

3,434,842

PHOTOGRAPHIC SILVER HALIDE EMULSIONS  
STABILIZED WITH 2-IMINO-THIAZOLONES  
Harald Hückstädt, Cologne-Stammheim, Wilhelm Saleck,  
Schildgen, Bergstrasse, Gladbach, Hans Ulrich and  
August Randolph, Leverkusen, and Herbert Grabhöfer,  
Cologne-Flittard, Germany, assignors to Agfa Gevaert  
Aktiengesellschaft, Leverkusen, Germany, a corporation  
of Germany

No Drawing. Filed July 19, 1965, Ser. No. 473,216  
Claims priority, application Germany, Aug. 8, 1964,  
A 46,797

Int. Cl. G03c 1/34

U.S. Cl. 96—109

5 Claims

## ABSTRACT OF THE DISCLOSURE

The invention relates to photographic silver halide emulsions which are sensitized by means of a chemical sensitizing agent having at least one polyoxyalkylene group and which are stabilized by means of 2-imino-thiazolone or -tetrahydrothiazinone compounds.

It is generally known that the sensitivity of photographic silver halide emulsions can be increased by adding suitable chemical compounds. Compounds of this type, referred to as chemical sensitizers, include, inter alia, polyalkylene oxides, in particular polyethylene oxides and their derivatives. The addition of such compounds increases the sensitivity and the contrast (gamma) of the silver halide emulsions.

Unfortunately, the use of polyalkylene oxides has the disadvantage that the fog level of the emulsions to which they are added is undesirably increased, with the result that sometimes they cannot be used.

As is generally known, fogging may be counteracted by adding so-called stabilizers or antifogging agents to the emulsions. Several compounds have already been used as stabilizers or antifogging agents, but unfortunately most of them have the disadvantage that they reduce the sensitivity and/or the contrast of the emulsion. Examples of such stabilizers include organic mercury compounds, heterocyclic mercapto compounds and azaindenes.

It has now been found that photographic silver halide emulsions which are chemically sensitized with polyalkylene oxides or their derivatives, may be stabilized against harmful fogging without impairing the original sensitivity or the gamma, by adding to the emulsions compounds of the general formula



in which R or R<sub>1</sub> represent hydrogen, alkyl preferably lower alkyl with up to 5 carbon atoms such as methyl or ethyl, aryl preferably phenyl, aralkyl such as benzyl or phenylethyl, or alkenyl, or R and R<sub>1</sub> together can form an ethylene group that completes an imidazoline ring; R<sub>2</sub> represents hydrogen, carboxyl, carbonylamide in which case the amide group may be substituted in particular with short-chain alkyl radicals with up to 5 carbon atoms, esterified carboxyl in particular with aliphatic alcohols containing up to 18 carbon atoms, preferably with those containing up to 5 carbon atoms, or with cycloaliphatic alcohols such as cyclohexanol; n is 0 or 1 and X represents any acid anion, preferably a halogen ion.

2

Of the compounds corresponding to the above general formula, those in which at least one of the substituents R, R<sub>1</sub> or R<sub>2</sub> is different from hydrogen, are preferred for the purposes of this invention. This applies in particular as regards the substituents R and R<sub>1</sub>. Where R<sub>1</sub> represents hydrogen, the stabilizers according to the invention may be tautomers according to the following equation:



The following compounds have proved to be particularly suitable:





The preparation of the Compounds I to X is described in "Zeitschrift für Angewandte Chemie," 74, page 906 (1962). The substances XIII and XIV are obtained by reacting the respective carboxylic acids with ethylamine. The Compound XV is prepared in accordance with the

prescription in the aforementioned paper while replacing hydrogen chloride by hydrogen bromide. Compounds of the type represented by the Formulae XI, XII, XVI to XXXI are obtained by reacting thiourea derivatives with chloroacetic acid or bromoacetic acid. This method is explained with reference to the following, specific example for Compound XII. This method is described in broad terms in the article by Lieberman and Lange in Liebigs Ann. 207, 128 (1881). As indicated by the above specific examples such compounds of the general formula in which  $n$  corresponds to 0 are prepared in which  $R_2$  stands for hydrogen.

#### Preparation of Compound XII

10.4 g. of N,N'-dimethylthiourea (0.1 mol) and 9.45 g. of chloroacetic acid (0.1 mol) are separately dissolved in methanol. The solutions are combined and refluxed for two hours. The methanol is then distilled off, leaving behind a yellowish crystalline mass from which pale yellowish crystals decomposing above 210° C. are obtained after recrystallization from methanol/ether.

In the case of silver halide emulsions mixed with polyalkylene oxides, the compounds of the present invention produce a marked reduction in fogging both when the emulsions are fresh and after they have been stored in a heating chamber.

The compounds of the present invention also have the effect of reducing fogging in cases where developing is carried out over a prolonged period.

The emulsions used are chemically sensitized with chemical sensitizers containing a polyalkylene oxide group, preferably a polyethylene oxide group, such as polyalkylene oxides or with polyalkylene oxide derivatives, particularly with polyethylene oxides or their derivatives. Examples of such polyethylene oxides are given in U.S. Patents Nos. 2,423,549 and 2,441,389.

Polyethylene oxide derivatives are obtained by condensing a polyethylene oxide with compounds containing an active hydrogen atom. Suitable organic compounds with active hydrogen atoms are for instance alcohols, primary or secondary amines, acids, amides and phenols, such as monohydric saturated or unsaturated alcohols having 1 to 20 carbon atoms, e.g., ethanol, dodecanol, stearyl alcohol and oleyl alcohol, polyhydric alcohols, e.g., glycols, glycerol, pentaerythritol, trimethylol propane, aliphatic primary or secondary amines, e.g., N-methyl-N-dodecylamine, aliphatic carboxylic acids, e.g., lauric acid, stearic acid, oleic acid or the amides of these acids, and phenol and alkyl phenols, e.g., p-dodecyl phenol. Preferred derivatives of polyalkylene oxides are reaction products of alkylene oxide or of their polymers with compounds containing hydrocarbon radicals with 10 to 10 carbon atoms. The quantity used will depend upon the silver halide content of the emulsion to which the compounds are added. It can vary from 0.01 g. to 1 g. per 1 kg. of silver halide emulsion. The preferred quantity being 0.05 to 2 g. per 1 mol of silver halide. The optimum quantity can easily be established empirically for each emulsion.

Suitable chemical sensitizers of the above type may be illustrated by the following formula:



wherein R stands for hydrogen, an aliphatic hydrocarbon radical (e.g., ethyl, dodecyl, oleyl), an acyl radical of an organic carboxylic acid (e.g., lauric acid, oleic acid), a phenyl radical (e.g., phenyl, p-dodecylphenyl) and  $n$ =an integer greater than about 30.

Examples of such polyalkylene oxides can be found in U.S. Patents Nos. 2,240,472 and 2,400,532. The preferred chemical sensitizers to be used according to the present invention are phosphorus-containing derivatives of polyalkylene oxides especially those disclosed in U.S. patent application Ser. No. 368,714, filed May 19, 1964, now U.S. Patent 3,385,708, granted May 28, 1968 and No. 379,738, 75

filed July 1, 1964, now U.S. Patent 3,385,704, granted May 28, 1968.

These compounds are either the condensation products of 1 mol of a spirocyclic pentaerythritol-di-(phosphoric acid monohalide) and 1 to 2 mols of a polyethylene glycol having between 3 and 100 ethylene oxide units, or the condensation products of 1 mol of a monoamido phosphoric acid derivative and 1 to 2 mols of a polyethylene glycol having 3 to 100 ethylene oxide units. These compounds may be represented by the following formulae:



15 wherein  $n$  stands for 3 to 100,  $x$  stands for 1 to 10 and R stands for hydrogen or for the group  $\text{H} \cdot \text{O} - \text{CH}_2 \cdot \text{CH}_2 \cdot \text{H}$  wherein  $n$  has the same meaning as above, and



wherein

20  $R_1$  represents alkyl, aryl, aralkyl,  
 $R_2$  represents hydrogen, alkyl, aryl, aralkyl, or  $R_1$  and  $R_2$  together represent the ring members necessary to complete a 5- or 6-membered heterocyclic ring,  
 $n$  is an integer between 3 and 100,  
 $m$  is an integer between 0 and 100,  
 $x$  has a value between 1 and 5.

In Belgian patent specification No. 621,607 similar stabilizing additives are used for the quick processing of silver halide emulsions.

In that case, the meaning of the term stabilizing differs from its significance in the context of the present invention. According to the Belgian patent specification, such compounds are used to convert the photosensitive silver halide into a nonphotosensitive complex form. For this purpose, the compounds in question are used in much large quantities than in the present invention, i.e., not less than 1 mole per mol of silver halide. As far as the present invention is concerned, these compounds cannot be used in such large quantities because they would produce an excessive loss of sensitivity and, at the same time, an increase in fogging.

In German patent specification No. 1,150,277 heterocyclic compounds of the type used according to the present invention are used in combination with elementary sulphur or compounds yielding sulphur, as chemical sensitizers. There is no reference in that patent specification to the effect of these compounds as stabilizers in emulsions containing as a chemical sensitizer a polyethylene oxide.

The combination of compounds according to the present invention is effective when used with all types of silver halide emulsions such as silver chloride emulsions, silver chlorobromide emulsions and silver iodochlorobromide emulsions, but preferably with silver halide emulsions the silver halide of which comprises silver bromide and up to 10 mol percent of silver iodide. The compounds may be added to the emulsion at any stage during its preparation, but preferably after it has been chemically ripened. They are used in quantities of 0.1 to 15 g., preferably 0.5 to 5 g. per mol of silver halide. The emulsions may be optically sensitized or nonsensitized and may contain color couplers. They may also be sensitized with noble metals such as gold salts. In addition to the additives according to the invention, the emulsions may contain other conventional additives such as antifogging agents, wetting agents, gelatin plasticizers or gelatin hardeners.

#### EXAMPLE 1

A panchromatically sensitized highly sensitive silver iodoform bromide emulsion (6 mol percent of silver iodide)

which contains 60 g. of silver halide per liter, is stabilized with 4-hydroxy - 6 - methyl-1,3,3a,7-tetraazaindene and in addition contains the usual wetting agents, for example saponin, and hardening agents such as formaldehyde and 0.16 g per liter of a polyalkylene oxide corresponding to the formula



5 0.16 g. per liter of a chemical sensitizer corresponding to the following formula:



10 is tested as described in Example 1. The results of the tests are given in the following Table II.

15 The preparation of the polyalkylene oxide corresponding to the above formula is described in U.S. Patent No. 3,169,863 under its Compound V.

TABLE II

| Stabilizer     | Amount added per litre of emulsion, g. | Fresh emulsion |       |           | 3 days' storage in heating chamber at 60° C. |       |           |
|----------------|----------------------------------------|----------------|-------|-----------|----------------------------------------------|-------|-----------|
|                |                                        | Sensitivity, ° | Gamma | Fog level | Sensitivity, °                               | Gamma | Fog level |
| Sample:        |                                        |                |       |           |                                              |       |           |
| A <sup>1</sup> |                                        | Standard       | 0.80  | 0.15      | Standard                                     | 0.80  | 0.23      |
| B <sup>1</sup> | 0.48                                   | do             | 0.75  | 0.15      | do                                           | 0.75  | 0.16      |
| C <sup>1</sup> | 0.48                                   | do             | 0.70  | 0.15      | do                                           | 0.70  | 0.17      |
| D <sup>1</sup> | 0.48                                   | do             | 0.75  | 0.13      | do                                           | 0.75  | 0.17      |

<sup>1</sup> Standard.

and is divided into three parts. Each part is then mixed with the quantities indicated in the following table of one of the stabilizers according to the present invention, and is then cast in the usual way onto a transparent substratum consisting of, for example, cellulose acetate, and dried. The polyalkylene oxide corresponding to the above formula is prepared according to the prescription given in German 30 patent specification No. 1,182,523.

## EXAMPLE 3

A highly sensitive silver iodobromide emulsion similar to that described in Example 1, except that, in place of the chemical sensitizer used in that example, it contains 0.16 g. per liter of a polyethylene oxide with 90 35 ethylene units, is tested as described in Example 1. The results are given in the following Table III.

TABLE III

| Stabilizer     | Amount added per litre of emulsion, g. | Fresh emulsion   |       |           | 3 days' storage in heating chamber at 60° C. |       |           |
|----------------|----------------------------------------|------------------|-------|-----------|----------------------------------------------|-------|-----------|
|                |                                        | Sensitivity, °   | Gamma | Fog level | Sensitivity, °                               | Gamma | Fog level |
| Sample:        |                                        |                  |       |           |                                              |       |           |
| A <sup>1</sup> |                                        | ( <sup>1</sup> ) | 0.55  | 0.22      | -1.5                                         | 0.55  | 0.33      |
| B <sup>1</sup> | 0.48                                   | +1.0             | 0.65  | 0.15      | ( <sup>1</sup> )                             | 0.65  | 0.18      |
| C <sup>1</sup> | 0.48                                   | ( <sup>1</sup> ) | 0.55  | 0.17      | ( <sup>1</sup> )                             | 0.50  | 0.20      |

<sup>1</sup> Standard.

Each sample is exposed behind a step wedge and then developed for about 8 to 10 minutes at 20° C. to approximately the same gamma value in the following developer mixture:

|                                | Grams |
|--------------------------------|-------|
| p-Methylaminophenol sulfate    | 3     |
| Sodium sulfite (anhydrous)     | 80    |
| Borax                          | 10    |
| Potassium bromide              | 0.5   |
| Made up with water to 1 liter. |       |

The relative sensitivity, gamma values and the fog level are determined by the usual methods. The results are given in the following Table I.

## EXAMPLE 4

50 Portions of a silver iodobromide emulsion of the type described in Example 1 are mixed with different chemical sensitizers and additives according to the present invention, as shown in the following Table IV, and are cast onto a transparent substrate, each forming a layer of equal 55 thickness thereon, and then dried. They are developed in a hard-type developer for 10 minutes at 20° C., until the gamma value is 2 to 3.

The developer has the following composition:

|                               | Grams |
|-------------------------------|-------|
| p-Methylaminophenol sulfate   | 5     |
| Sodium sulfite (anhydrous)    | 40    |
| Hydroquinone                  | 6     |
| Potassium carbonate           | 40    |
| Potassium bromide             | 3     |
| Water to make up to 1,000 ml. |       |

TABLE I

| Stabilizer     | Amount added per litre of emulsion, g. | Fresh emulsion   |       |           | 3 days' storage in heating chamber at 60° C. |       |           |
|----------------|----------------------------------------|------------------|-------|-----------|----------------------------------------------|-------|-----------|
|                |                                        | Sensitivity, °   | Gamma | Fog level | Sensitivity, °                               | Gamma | Fog level |
| Sample:        |                                        |                  |       |           |                                              |       |           |
| A <sup>1</sup> |                                        | ( <sup>1</sup> ) | 0.70  | 0.16      | -1.5                                         | 0.65  | 0.19      |
| B <sup>1</sup> | 0.48                                   | +0.5             | 0.70  | 0.10      | -1.0                                         | 0.65  | 0.13      |
| C <sup>1</sup> | 0.48                                   | +0.5             | 0.75  | 0.10      | -1.0                                         | 0.65  | 0.13      |

<sup>1</sup> Standard.

The results of the tests are given in the following Table IV:

3. A photosensitive material as claimed in claim 2, wherein  $R_1$  represents alkyl.

TABLE IV

| Stabilizer<br>(0.48 g./<br>litre of<br>emulsion) | Sensitizer (0.16<br>g./litre of emulsion) | Fog level<br>after 5 minutes'<br>development | Fog level<br>after 10<br>minutes'<br>development |
|--------------------------------------------------|-------------------------------------------|----------------------------------------------|--------------------------------------------------|
| Sample:                                          |                                           |                                              |                                                  |
| A <sup>1</sup>                                   | XII                                       | As in Example 1                              | 0.17                                             |
| B                                                | XII                                       | do                                           | 0.11                                             |
| C                                                | VI                                        | do                                           | 0.11                                             |
| A <sup>1</sup>                                   |                                           | As in Example 2                              | 0.22                                             |
| B                                                | I                                         | do                                           | 0.18                                             |
| C                                                | II                                        | do                                           | 0.23                                             |
| D                                                | IX                                        | do                                           | 0.16                                             |
| A <sup>1</sup>                                   |                                           | As in Example 3                              | 0.31                                             |
| B                                                | XII                                       | do                                           | 0.18                                             |
| C                                                | VI                                        | do                                           | 0.20                                             |

**1 Standard.**

We claim:

1. In a photosensitive photographic material which comprises at least one silver halide emulsion layer containing a chemical sensitizer having a polyalkylene oxide group, the improvement according to which said emulsion layer has added thereto in stabilizing quantities a stabilizer of the general formula



wherein

R and R<sub>1</sub> represent hydrogen, alkyl, aryl, aralkyl or alkenyl, 40

$R_2$  represents hydrogen, carboxyl, carbonylamide or esterified carboxyl,

$n$  is 0 or 1, and

X represents any acid anion.

2. A photosensitive material as claimed in claim 1,  
wherein at least one of the substituents R, R<sub>1</sub> or R<sub>2</sub> is different from hydrogen. 4

20 4. A photosensitive material as claimed in claim 3,  
wherein the stabilizer corresponds to the formula



5. A photosensitive material as claimed in claim 1  
30 wherein R and R<sub>1</sub> represent hydrogen, alkyl having up  
to 5 carbon atoms, phenyl, benzyl or phenylethyl, R<sub>2</sub>  
represents hydrogen, carboxyl, carbon amide, alkyl sub-  
stituted carbon amide having up to 5 carbon atoms in  
each alkyl group, esterified carboxyl having up to 18 car-  
bon atoms or cycloalkyl.

### References Cited

UNITED STATES PATENTS

- |           |        |                              |        |
|-----------|--------|------------------------------|--------|
| 2,131,038 | 9/1938 | Brooker et al. -----         | 96-109 |
| 3,189,453 | 6/1965 | Herz et al. -----            | 96-61  |
| 3,321,312 | 5/1967 | Muller-Bardorff et al. ----- | 96-109 |

NORMAN G. TORCHIN, *Primary Examiner.*

J. R. EVERETT, *Assistant Examiner.*

U.S. CL. X R